

## UNITED STATES PATENT OFFICE

2,273,312

## TREATMENT OF GASOLINE

Joseph A. Chencsek, Chicago, Ill., assignor to  
 Universal Oil Products Company, Chicago, Ill.,  
 a corporation of Delaware

No Drawing. Application June 28, 1940.  
 Serial No. 342,951

2 Claims. (Cl. 44—9)

This invention relates to a method for improving the stability of hydrocarbon distillates insofar as color and gum formation are concerned. More particularly the process concerns improved methods of preventing deterioration of cracked gasolines which may be stored over relatively long periods of time in the presence of air.

The use of inhibitors to prevent the depreciation of olefin-containing hydrocarbon distillates such as cracked gasoline has been practiced. Such compounds as alkyl-substituted phenols, aminophenols, fractions of wood tar distillates, etc., have been added to cracked gasoline in relatively minor quantities, of the order of 0.001—0.10% to inhibit the formation of objectionable oxidation products and prevent loss of color and antiknock properties of said gasolines during storage periods. The use of inhibitors has replaced or supplemented such forms of refining as acid-treating, clay treating and the like. The result has been a material saving in refining costs as well as the conservation of substantial amounts of gasoline which were formerly lost in the refining steps.

The present invention offers a means of improving the inhibiting properties of gasoline gum inhibitors and of effecting material savings in the quantities of such materials which may be required adequately to preserve the valuable properties of gasoline.

In one specific embodiment the present invention comprises a method for treating olefin-containing hydrocarbon distillate to preserve the valuable properties thereof by adding to said distillate a gasoline gum inhibitor together with a relatively minor quantity of a condensation product of an aliphatic aldehyde with ammonia.

An example of such a compound is aldehyde ammonia ( $\text{CH}_3\text{CH}(\text{OH})\text{NH}_2$ ). Other similar related compounds of aliphatic aldehydes and ammonia may be used, although the compounds are not necessarily equivalent in their action.

The quantity of aldehyde ammonia commonly used in the gasoline is of the order of 0.0001—0.01%. The exact quantity required is a function of the inhibitor used and of the gasoline as well as the desired stability of the gasoline treat-

ed. The aldehyde ammonia are not of themselves gum inhibitors and the effect observed is not, therefore, such as might be expected by the mixing of two gasoline gum inhibitors. When added alone to cracked gasoline in amounts up to approximately 0.1%, little or no increase in the oxygen bomb induction period is to be observed and storage tests indicate that no protection is obtained for the gasoline under storage conditions. However, when a gum inhibitor is present, the induction period with a given quantity of inhibitor is markedly increased and with some of the more effective aldehyde-ammonias, more than equal weight percentages of the inhibitor can be replaced without suffering a loss in inhibitor potency. This will be brought out more fully in the example.

The following example is given to illustrate the usefulness and practicability of the process, but should not be construed as limiting it to the exact conditions or compounds described therein.

A Pennsylvania cracked gasoline had an induction period of 115 minutes which was increased to 330 minutes by the addition of 0.008% of N-butyl-p-aminophenol. Upon the addition to the inhibited gasoline of 0.005% of aldehyde ammonia, the induction period was increased to 415 minutes.

I claim as my invention:

30 1. In the stabilization of olefinic gasoline by the addition of gum inhibitors thereto, the method of increasing the effectiveness of the inhibitor which comprises incorporating into the gasoline, in addition to the gum inhibitor, a condensation product of an aliphatic aldehyde with ammonia, the quantity of said product being insufficient, in the absence of said inhibitor, to effect any appreciable gum inhibition of the gasoline.

2. In the stabilization of olefinic gasoline by 40 the addition of gum inhibitors thereto, the method of increasing the effectiveness of the inhibitor which comprises incorporating into the gasoline, in addition to the gum inhibitor, a quantity of aldehyde ammonia which is insufficient, in the absence of said inhibitor, to effect any appreciable gum inhibition of the gasoline.

JOSEPH A. CHENICEK.